

## UNITED STATES PATENT OFFICE.

FREDERICK GEORGE EDBROOK, OF HAMMERSMITH, LONDON, ENGLAND.

## LACQUER FOR SHOE HEELS AND THE LIKE.

No Drawing. Application filed July 11, 1923, Serial No. 650,961, and in Great Britain July 26, 1922.

This invention relates to lacquers for shoe heels and the like, and it consists of an improved composition for application to wooden heels in order to produce a fine enamelled 5 finish.

This lacquer comprises cellulose acetate, dichlorhydrin, and solvents, including alcohol.

The lacquer is composed preferably of the 10 following materials, in proportional parts of weight:

|                    | Parts. |
|--------------------|--------|
| Industrial alcohol | 7      |
| Dichlorhydrin      | 10     |
| Lithopone          | 48 55  |

Two coats of this filler solution will be sufficient to fill the grain of the wood.

The heels are then allowed to dry thoroughly and are then buffed smooth with fine glass-paper and are ready for the application of the lacquer previously described in this specification.

The prepared wooden heels are now given successive coats of the lacquer with a camel hair brush or they may be sprayed with the lacquer with a fine spray worked by means of compressed air, allowing a few minutes between each coat for drying. Four coats should be found sufficient if the heels are perfectly smooth, but a finer finish can be obtained by adding further coats, until by test the desirable number of coats has been determined, according to the conditions and the finish required.

When a sufficient number of coats have been applied, the heels are allowed to harden for about 12 hours, and they are then well buffed with a cloth bob and polishing wax on a buffering machine until the desired finish is obtained.

Having thus described my invention, what I claim is:

1. A lacquer for shoe heels and the like consisting of substantially equal proportions of cellulose acetate and dichlorhydrin, and a solvent thereof, said solvent comprising substantially one part of benzyl alcohol, two parts of industrial alcohol, five parts of benzol, and four-hundred parts of acetone.

2. A lacquer for shoe heels and the like, composed substantially of cellulose acetate 12 parts, acetone 1152 parts, benzol 14 parts, benzyl alcohol 3 parts, industrial alcohol 7 parts, and dichlorhydrin 10 parts.

3. A lacquer adapted to afford a fine finish to shoe heels, comprising cellulose acetate and dichlorhydrin combined in substantially equal parts, and a solvent thereof, said solvent including alcohol.

20 Such a composition may be mixed, for example, in an earthenware jar, fitted with a mechanical or other stirring or agitating device. The cellulose acetate is first put in the jar and the acetone added: this is agitated until it becomes a liquid solution. The dichlorhydrin and benzol are then added and the solution is agitated for 15 minutes, when finally the benzyl alcohol and industrial spirit are added, and the solution agitated for a further 15 minutes.

25 The solution is next strained through fine cloth and decanted and is then ready for use.

30 Before applying the lacquer made in accordance with the foregoing directions, the wooden heels should be buffed until they are perfectly smooth, all imperfections being taken out by the buffing. This is most im-

35 portant if a fine enamelled finish is required. After the heels have been buffed perfectly smooth, it is preferable that a preliminary lacquer or filler solution be used to fill all the grain of the wood.

40 This filler solution (or preliminary lacquer) may be, with advantage, composed of:

|                   | Parts. |
|-------------------|--------|
| Cellulose acetate | 12     |
| Acetone           | 1152   |
| Benzol            | 14     |
| Benzyl alcohol    | 3      |

FREDERICK GEORGE EDBROOK.